

## UNITED STATES PATENT OFFICE.

HARRY A. SCHWARTZ, OF CLEVELAND, OHIO, ASSIGNOR TO NATIONAL MALLEABLE AND STEEL CASTINGS COMPANY, OF CLEVELAND, OHIO, A CORPORATION OF OHIO.

## MAKING MALLEABLE-IRON CASTINGS.

No Drawing. Application filed October 30, 1924. Serial No. 746,870.

In the manufacture of malleable iron castings it is customary to have silicon present in the iron before casting so that, in the subsequent malleabilizing operation, it may 5 assist the decomposition or breaking up of the cementite in the iron. After casting and while the casting is cooling the presence of too much silicon, however, causes the precipitation during or just after freezing of 10 a percentage of the carbon in the flaky form normally found in grey iron castings and renders the castings worthless for conversion into malleable iron, and owing to this 15 action the amount of silicon present or to be added must be regulated with very great care. I have found that the addition of small proportions of a graphitization accelerating such as zirconium to iron containing an inappreciable percentage of silicon 20 greatly accelerates the annealing cycle of such malleable iron, acting in much the same way as larger amounts of silicon, but without the deleterious effects of silicon.

In carrying out my invention I have 25 found that iron containing no substantial percentage of silicon and to which is added a small amount of zirconium (approximately .50% or less of zirconium being sufficient in the annealed casting) may be cast without precipitating the carbon, and when annealed graphitizes as completely and more satisfactorily than malleable iron of normal analysis which contains substantially .70-.80% of silicon and no zirconium. Suitable larger amounts may be added to promote still further ease of annealing. In fact, the limit of the amount of zirconium which may be added is that which will cause primary precipitation of graphite, and such 35 limit varies with the shape and thickness of the castings. I have found, however, that castings containing after annealing approximately .20% or less of zirconium graphitize completely and satisfactorily. Similar additions in properly reduced amount can be made to metal having the silicon content equal to or less than that normally present in malleable iron. Such additions, even in amounts as small as .10% or less, will similarly benefit the metal with respect to its annealing properties, resulting in a marked reduction of the time required for anneal.

The effect of silicon in iron for malleable

castings is to raise the critical point above which carbon is soluble and to lower the 55 solubility of free carbon in solid iron at all temperatures above the critical point just mentioned. Silicon thus acts by decreasing the solubility of carbon in the iron and renders graphitization during annealing at a 60 given temperature more rapid and complete, but by reason of its completeness there is danger of precipitation of carbon while cooling in the mold, which is ordinarily known as primary graphitization. Thus, if substantial amounts of primary graphite are present (for instance, as much as .10% or even less) the properties of the annealed casting are so far deteriorated as to practically destroy its commercial value. Zirconium in the small amounts contemplated, on the other hand, so far as I have observed, has no appreciable effect on the critical point of the alloy.

My invention is particularly adapted for 75 use in making malleable castings with comparatively heavy sections, since the slow cooling of such castings in the casting operation, because of their thick sections, tends to permit the precipitation of the carbon in flaky form if the castings contain too high a percentage of silicon. A result of using a graphitization accelerator such as zirconium is to shorten the annealing cycle and therefore decrease the time during which 80 the surface of the castings is exposed to the decarbonizing effects of air or of the packing material which is in contact with such surface, so that the thickness of the ferrite skin on the castings formed by such exposure is lessened by the shortening of the time of exposure. As this ferrite skin is 85 more difficult to machine than the material underneath, a definite improvement in machining qualities is thus achieved.

My invention is also useful in the manufacture of malleable iron castings in which increased strength may be obtained by the addition of small percentages of metals such as chromium, as the zirconium and other 100 metals which act similarly, such as titanium and uranium, have the effect not only of offsetting the very great and prohibitive increase in the time required for annealing, which is the usual result of additions such 105 as chromium, but also assisting in the graph-

itization of the casting. The chromium also adds valuable rust and oxidization resisting qualities to the iron.

The terms and expressions which I have employed are used as terms of description and not of limitation, and I have no intention, in the use of such terms and expressions, of excluding any equivalents of the features shown and described, or portions thereof, but recognize that various modifications are possible within the scope of the invention claimed, it being understood that by the use of the term "graphitization accelerator" I refer to such elements as assist in the graphitization of the metal during annealing.

What I claim is:

1. The process of making malleable iron castings containing an inappreciable percentage of silicon, which comprises adding a small amount of zirconium as a graphitization accelerator, casting the metal without precipitating a substantial proportion of the carbon, annealing the casting and thereby precipitating the carbon in the form of small particles.

2. The process of making malleable iron castings which comprises adding a small percentage of zirconium to the iron, annealing the casting and thereby effecting graphitization of the casting.

3. The process of making malleable iron castings, which comprises adding to the iron, such a percentage of zirconium as will produce less than one-half of one per cent of zirconium in the annealed casting, annealing the casting and thereby effecting the graphitization of the casting.

4. The process of making malleable iron castings which comprises adding a small percentage of zirconium to the iron and also a strengthening element, annealing the casting and thereby effecting graphitization of the casting, the zirconium overcoming the retarding effect of the strengthening element upon the annealing operation, and also assisting in the graphitization of the casting.

5. The process of making malleable iron castings which contain, in addition to the elements usually present in malleable iron, a strengthening element which retards annealing, adding to such iron while molten an element such as zirconium, titanium or uranium which accelerates annealing, such element overcoming the retarding effect of the strengthening element and also assisting in the graphitization of the casting, annealing the casting and thereby precipitating the carbon in the form of small particles.

HARRY A. SCHWARTZ.